

Dec. 22, 1953

R. R. LLOYD ET AL

2,663,686

PRODUCTION OF ELECTROLYTIC CHROMIUM FROM FERROCHROME

Filed July 24, 1951



## UNITED STATES PATENT OFFICE

2,663,686

## PRODUCTION OF ELECTROLYTIC CHROMIUM FROM FERROCHROME

Rex R. Lloyd, Joe B. Rosenbaum, and Vernon E. Homme, Boulder City, Nev., assignors to the United States of America as represented by the Solicitor of the Department of the Interior

Application July 24, 1951, Serial No. 238,362

5 Claims. (Cl. 204—105)

(Granted under Title 35, U. S. Code (1952), sec. 266)

1

The invention described herein may be manufactured and used by or for the Government of the United States for governmental purposes without the payment to us of any royalty thereon in accordance with the provisions of the Act of April 30, 1928 (Ch. 460, 45 Stat. L. 467).

This application relates to the production of electrolytic chromium from ferrochrome and more particularly to a process for obtaining an electrolyte produced from ferrochrome for an electrolytic cell from which pure chromium metal or chromium containing minor quantities of iron is to be obtained.

This application is related to copending applications of Rex R. Lloyd and Joe B. Rosenbaum entitled "Electrolytic Diaphragm Cell," Serial No. 238,361, filed July 24, 1951; Rex R. Lloyd and Vernon E. Homme entitled "Electrodeposition of Chromium and Electrolyte Therefor," Serial No. 238,360, filed July 24, 1951; and Rex R. Lloyd and Joe B. Rosenbaum entitled "Anode for Electro-winning Chromium Metal," Serial No. 238,363, filed July 24, 1951.

Chromium for metallurgical purposes is ordinarily processed by smelting ores which contain a high, such as three to one, ratio of chromium to iron in an electric furnace with a carbonaceous reducing agent to produce high carbon ferrochrome. For certain purposes, such as production of stainless steel, carbon cannot be tolerated with the chromium except to a very limited extent so the high carbon ferrochrome is further processed with chrome-silicon, or the like, to produce low carbon ferrochrome.

Nearly all domestic ores, however, do not contain a sufficiently high ratio of chrome to iron to produce ferrochrome containing 68 to 70 per cent chromium, which is demanded by present metallurgical practice. The problem which led to the invention, therefore, was to remove the iron and carbon from high carbon ferrochrome produced by conventional and well-known methods from low-grade domestic chromite ores.

An object of this invention is to provide a method of producing substantially pure electrolytic chromium or chromium containing minor quantities of iron from ferrochrome.

An additional object of the invention is to produce electrolytic chromium by a process which is less costly than the heretofore customary processes by which electrolytic chromium is prepared from chromic acid or by the aluminum or silicon reduction of chromic oxide which in turn was prepared from sodium dichromate.

Further objects and advantages of the inven-

tion will be appreciated from a consideration of the following detailed description of the invention.

The figure of the drawing is a flow sheet of the preferred process of the invention.

In one embodiment of the invention, and referring now to the flow sheet, the process starts with ferrochrome which may be prepared from chromite ores by reduction with a carbonaceous reducing agent in an electric furnace in accordance with well-known procedures. See, for example, Mellor, "A Comprehensive Treatise on Inorganic and Theoretical Chemistry," vol. XI, page 455. Ordinarily high-carbon ferrochrome is used because of cost, but the process is equally applicable to any alloy containing chromium and iron which can be dissolved in acid. Ferrochrome ordinarily contains major quantities of chromium, iron, silicon, and carbon, and minor quantities of several other metals such as nickel, cobalt, and vanadium.

According to the invention, ferrochrome is dissolved in a hot solution containing sulfuric acid. As shown in the flow sheet, this solution is preferably the return depleted chrome liquor which is enriched with sufficient sulfuric acid to make up for losses in the process. This depleted chrome liquor is primarily a solution of sulfuric acid, and it also contains ammonia or ammonium sulfate and minor quantities of iron sulfate and chromium sulfate. The major portion of the acid required for the treatment of the ferrochrome is present in the depleted chrome liquor and, preferably, an excess of acid is used and recycled with the chrome liquor.

It has been discovered that ferrochrome will not dissolve in acid liquor which contains hexavalent chromium or trivalent iron. It is, therefore, essential that the leach liquor used to treat the ferrochrome be substantially free of both chromium and iron of these higher valences.

When ferrochrome is dissolved in sulfuric acid, the chromium is converted principally to chromic sulfate with some chromous sulfate; iron is converted to ferrous sulfate. Some of the metallic impurities also enter the solution in various forms. The temperature of the leach is not critical, but the reaction rate is increased by increasing the leach temperature.

The leach liquor is filtered to remove any residue of the ferrochrome, such as silica and the filtrate goes to a conditioning tank. This filtrate contains free sulfuric acid, chromium sulfate, iron sulfate and ammonium sulfate.

The liquor in the conditioning tank is held at a

temperature of from 60° to 80° C., the latter temperature, 80° C., being preferred, for at least two hours and preferably from 8 to 24 hours. This conditioning step at 80° C. functions to maintain the chromium in the solution in the "green" or hydrolyzed modifications in which forms it has a high solubility and does not form alums, and at the same time the iron appears to de-hydrolyze during conditioning, permitting the formation of ferrous ammonium sulfate crystals upon cooling the liquor following conditioning.

If the conditioning step is omitted, ferrous ammonium sulfate crystals will form to only a limited extent, if at all, upon subsequent cooling. This is particularly true if the ferrochrome leach has taken place at temperatures in excess of 90° C. As stated above, conditioning may be performed at 60° C. to 80° C. However, at the lower temperatures, chromium reversion to the "violet" modification is accelerated, resulting in increased chromium alum precipitation with the ferrous ammonium sulfate crystals in the subsequent step of the process. If the leach is carried out at 80° C. plus or minus 10° C., then separate conditioning is less necessary but the conditioning step has, nevertheless, been affected.

Crystallization is accomplished by cooling the conditioned liquor to a low temperature. Preferably, the liquor is cooled to 10° C. or less. This cooling causes precipitation of ferrous ammonium sulfate,  $(\text{NH}_4)_2\text{SO}_4 \cdot \text{FeSO}_4 \cdot 6\text{H}_2\text{O}$ , and a small quantity of chromium ammonium alum,



Impurities, such as nickel, cobalt, and titanium, which are dissolved from the ferrochrome, are also removed in these crystals.

These crystals are filtered from the liquor, and the thus purified liquor substantially comprises sulfuric acid, chromium sulfate, and ammonium sulfate. The purified liquor still contains a small amount of iron sulfate as well as small quantities of any other impurities present in the leach liquor, but these do not precipitate in the subsequent aging step and eventually build up in the system until they do come out with the ferrous ammonium sulfate crystals formed in the above-mentioned cooling and crystallizing step.

The purified liquor thus obtained is heated and held at a temperature above normal room temperature, with a temperature of approximately 30° C. being preferred. During this aging, the chromic sulfate is converted from the hydrolyzed and green modifications, which do not form alums, to the violet modification where alum forms and precipitates. The pH of the liquor must be below 1.2 and preferably a range of pH of 0 to 0.5 is used. It is essential to the production of an adequately pure chrome alum that the iron and other impurities be removed in the crystallization step at a temperature substantially lower, such as 25° C. or below, than the temperature at which the chrome alum is precipitated.

The chrome alum is used for the production of electrolytic chromium as described in the above-mentioned copending application Serial No. 238,360, filed July 24, 1951. The catholyte overflow from the cell contains chromic sulfate, chromous sulfate and ammonium sulfate and is returned directly to the liquor aging tank. The anolyte overflow contains hexavalent chromium, ammonium sulfate, free sulfuric acid and a small amount of trivalent chromium. This anolyte overflow is treated with a suitable reducing agent, such as sugar, ammonia, sulfur dioxide or the like,

in order to reduce the hexavalent chromium in the anolyte. The anolyte overflow, after reduction, is also returned to the liquor aging tank.

These liquors are returned to the aging tank since they are free of impurities and they help to dilute the impurity concentration in the aging tank. By impurities is meant any constituent other than chromium, ammonium sulfate or sulfuric acid. As stated above, any of several well-known reducing agents, such as sugar, ammonia, sulfur dioxide and the like, can be used to reduce the hexavalent chromium in the anolyte overflow. If the anolyte is heated to 250° C. or above in an autoclave, the chromic acid will spontaneously decompose according to the following reaction:



If sulfur dioxide is used for a reducing agent, very little make-up sulfuric acid is required by the process. Evaporation is, practically speaking, necessary somewhere in the flow sheet to remove excess water. If the anolyte overflow is evaporated to a specific gravity of 1.6 or above, a large part of the hexavalent chromium separates out as a crude chromic acid, which can be purified by well-known means. If the chromic acid is not removed, the evaporation step can be accomplished elsewhere in the flow sheet, such as with the leach step, without changing the essential features of the process.

As shown in the flow sheet, the ferrous ammonium sulfate crystals may be recrystallized to recover the chromium or they may be discarded. Conditioning, in the flow sheet, means heating the solution to about 80° C. to stabilize the chromium in the green modifications so that it will not subsequently precipitate with the iron. The final iron crystals may be treated by conventional methods to recover ammonia or ammonium sulfate, for return to the system as chrome liquor, as shown in the flow sheet, or they may be otherwise utilized or discarded without changing the essential features of the process.

It will be appreciated that the procedure of recycling of solutions in the novel manner disclosed herein improves the economics of the process by minimizing the losses and by accelerating reactions through control of chemical compositions. Thus the catholyte overflow is returned to the process to prevent the loss of chromium and ammonia; the treated anolyte overflow is returned in order to save its chromium, ammonia and acid. In addition, return of these highly pure liquors serves to dilute the impurity concentration in the chromium aging liquor, thus reducing the quantity of impurities tending to precipitate with the chromium alum. The depleted chromium liquor, from which the alum has precipitated, is returned to the process in order to utilize its acid content for ferrochrome dissolution, its ammonia in raising the ammonia concentration of the leach liquor high enough to remove iron in the subsequent iron crystallization step, and its chromium to increase the chromium concentration to the range in which precipitation of chromium alum is rapid during the aging step. Dilution of the chromium aging liquor with return catholyte overflow and reduced anolyte overflow is desirable to reduce the impurities in the precipitated chrome alum. It will be appreciated, however, that applicants' process may be operated without the recycling steps without departing from the spirit and scope 75 of the invention.

The following example is illustrative of one particular embodiment of the process of the invention.

## EXAMPLE

## Experimental data

A 160-pound batch of minus  $\frac{1}{8}$  inch high-carbon ferrochrome was leached for 48 hours with 407 gallons of depleted chromium liquor fortified with 80 pounds of 93-per cent sulfuric acid. The ferrochrome contained approximately 64 per cent chromium, 25 per cent iron, 6 per cent carbon, and 3 per cent silicon. The depleted chromium liquor contained 20 grams chromium, 2.2 grams iron, 52 grams ammonia, and 200 grams free sulfuric acid per liter. The leach temperature was maintained at 95° to 100° C. and the evaporation was controlled, by means of a condenser on the leach kettle, to 102 gallons of water.

At the end of the 48 hours the leach was filtered hot through a lead filter press. The filter press residue weighed 15 pounds wet and consisted mostly of silica with a small quantity of carbon and contained 2 pounds of chromium and 0.5 pound of iron. The filtrate measured 302 gallons and analyzed 67 grams chromium, 19 grams iron, 70 grams ammonia (all present as the sulfates), and 155 grams free sulfuric acid per liter.

To the 302 gallons of filtrate was added 69 gallons of chrome liquor obtained by recrystallization of the chromium containing ferrous ammonium sulfate from a previous batch. The recovered chrome liquor analyzed about 22 grams chromium, 4 grams iron, and 62 grams ammonia per liter, all present as sulfates. The 371 gallons of mixed chromium liquor was then conditioned by holding at 80° C. for 16 hours.

The conditioned liquor was next cooled to 5° C. in a vacuum crystallizer where ferrous ammonium sulfate and other crystals formed. These crystals were separated from the purified liquor in a perforate-type basket centrifuge. The crystals weighed 450 pounds and analyzed about 9 per cent iron, 3 per cent chromium, and 8 per cent ammonia. The purified liquor analyzed 62 grams chromium, 3 grams iron, 65 grams ammonia per liter and measured 323 gallons.

The impure crystals were dissolved in 57 gallons of water along with 100 pounds of ammonium sulfate and the chromium was stabilized by conditioning at 80° C. for 4 hours. The liquor was cooled to 5° C. and the crystals separated as in the first crystallization, to yield 300 pounds of crystals and 69 gallons of liquor. The final crystals analyzed 13 per cent iron, 0.2 per cent chromium, and 8.5 per cent ammonia. The recovered chrome liquor analyzed the same as the 69 gallons previously added to the leach liquor and was recycled to the next batch.

The purified chromium liquor obtained from the first crystallization was pumped to a continuously aging thickener containing about 4,000 gallons of depleted liquor. The aging liquor was held at 32° to 35° C. and the alum crystals which formed were separated in a perforate-type centrifuge, with the liquor returning to the aging tank. Approximately 1,330 pounds of chrome alum were produced from this particular batch. The wet alum analyzed 10.6 per cent chromium, 0.03 per cent iron, and 3.4 per cent ammonia. A 407-gallon batch of depleted chrome liquor was removed from the aging thickener and returned to the next batch.

The 1,330 pounds of chrome alum was dissolved

75

in 37 gallons of water at 70° C. to make a cell feed solution containing about 130 grams chromium, 0.4 gram iron, and 42 grams ammonia per liter. This cell feed was fed to a continuously operating cell having five stainless steel cathodes with a submerged area of 37.5 square feet. The catholyte solution analyzed 17 grams trivalent chromium, 23 grams divalent chromium, and 30 grams ammonia per liter. The cell feed was added at such a rate that the analysis of the catholyte solution remained constant throughout the test. A current of 3,000 amperes on the cell, at a potential of 4.7 volts, electrodeposited 101 pounds of electrolytic chromium from the catholyte solution in 39 hours. The metal analyzed 99.3 per cent chromium, and 0.4 per cent iron. Of the 141 pounds of chromium entering the cell in the cell feed, 100 pounds were electrodeposited, 11 pounds left the cell in 35 gallons of catholyte overflow, and 30 pounds in 140 gallons of anolyte overflow. The anolyte overflow analyzed 3 grams trivalent chromium, 22 grams hexavalent chromium, 19 grams ammonia, and 300 grams free sulfuric acid per liter. About 60 gallons of water was added to the anolyte, during the test, to keep the specific gravity lower than the catholyte. The electrolytic cell operated at 60° C. and a pH of 2.5 to 2.6 during the test.

The catholyte overflow was returned directly to the liquor-aging step where the divalent chromium maintained completely reducing conditions in the aging tank. If a small quantity of divalent chromium, or other strong reducing agent, is not added to the liquor-aging step the ferrous iron will oxidize to give a trace of ferric iron which, in turn, adversely affects the rate of alum formation and the purity.

The anolyte overflow solution was maintained at 60° C. while the hexavalent chromium was reduced by adding 11 pounds of sugar. The reduced anolyte was then returned to the liquor-aging tank.

It will be appreciated from a reading of the foregoing specification that the invention herein described is susceptible of various changes and modifications without departing from the spirit and scope thereof. The invention is, therefore, to be limited only by the scope and spirit as set forth in the appended claims.

## What is claimed is:

1. A process for production of electrolytic chromium from ferrochrome comprising leaching said ferrochrome with a hot acidic solution containing chromium depleted liquor from a subsequent stage of the process to thereby form a solution containing chromium sulfate, ammonium sulfate, and iron sulfate, crystallizing the bulk of the iron from said solution in the form of ferrous ammonium sulfate, mixing the remaining liquor with an anolyte effluent solution and a catholyte effluent solution containing chromic sulfate, chromous sulfate, ammonium sulfate, and sulfuric acid, aging the resulting liquor at a pH below 1.2, crystallizing chromium ammonium sulfate from the aged liquor at a temperature higher than that at which said ferrous ammonium sulfate was crystallized, recycling the chromium depleted liquor to provide a substantial portion of the acid solution for leaching said ferrochrome, utilizing the crystallized chromium ammonium sulfate with water to form an electrolyte feed solution, electrolyzing said solution in an electrolytic compartment cell in which chromium is plated from the solution and in which anolyte effluent containing hexavalent chromium, am-

monium sulfate, and sulfuric acid and catholyte effluent containing chromium sulfate, chromous sulfate and ammonium sulfate are produced, reducing the hexavalent chromium of the anolyte effluent to lower valence forms, and recycling said reduced anolyte solution and said catholyte solution for admixture with the chrome liquor from which ferrous ammonium sulfate has been removed.

2. The process of claim 1 in which the hexavalent chromium in said anolyte solution is reduced by heating the anolyte solution to 250° C.

3. A process for production of electrolytic chromium from ferrochrome comprising leaching said ferrochrome with a hot acidic solution containing chromium depleted liquor from a subsequent stage of the process to thereby form a solution containing chromium sulfate, ammonium sulfate, and iron sulfate, crystallizing the bulk of the iron from said solution in the form of ferrous ammonium sulfate, mixing the remaining liquor with an anolyte effluent solution and a catholyte effluent solution containing chromic sulfate, chromous sulfate, ammonium sulfate, and sulfuric acid, aging the resulting liquor at a pH below 0.5 at a temperature of about 30° C., crystallizing chromium ammonium sulfate from the aged liquor at a temperature higher than that at which said ferrous ammonium sulfate was crystallized, recycling the chromium depleted liquor to provide a substantial portion of the acid solution for leaching said ferrochrome, utilizing the crystallized chromium ammonium sulfate with water to form an electrolyte feed solution, electrolyzing, said solution in an electrolytic compartment cell in which chromium is plated from the solution and in which anolyte effluent containing hexavalent chromium, ammonium sulfate, chromous sulfate and ammonium sulfate are produced, adding a reducing agent to said anolyte effluent thereby reducing the hexavalent chromium of the anolyte solution to lower valence forms, and recycling said anolyte solution and said catholyte solution for admixture with the chrome liquor from which ferrous ammonium sulfate has been removed.

4. The process of claim 3 in which the added reducing agent is sugar.

5. A process for the production of electrolytic chromium from ferrochrome comprising leaching said ferrochrome with a hot aqueous solution

10 15 20 25 30 35 40 45 50

containing sulfuric acid, ammonium sulfate, and chromium compounds substantially free of hexavalent chromium and trivalent iron, recycled from a subsequent stage of the process, to thereby form a solution containing chromium sulfate, ammonium sulfate and iron sulfate, filtering the thus formed liquor to remove insoluble constituents therefrom, cooling the liquor to a temperature of from about 60° C. to 80° C. for a period of two to twenty-four hours to maintain the chromium in solution in a hydrolyzed form and to dehydrolyze the iron in solution, cooling the thus conditioned liquor to a temperature below 25° C. thereby causing precipitation of the bulk of the iron as ferrous ammonium sulfate crystals, filtering said liquor to remove said crystals, mixing the remaining liquor with anolyte effluent solution and catholyte effluent solution containing chromic sulfate, chromous sulfate, ammonium sulfate and sulfuric acid, aging the resulting liquor at a pH of below 1.2 and at a temperature of about 30° C., crystallizing chromium ammonium sulfate from the aged liquor, recycling the chromium depleted liquor to the leaching step with make up sulfuric acid, utilizing the crystallized chromium ammonium sulfate with water to form an electrolyte feed solution, electrolyzing said solution in an electrolytic compartment cell in which chromium is plated from the solution and in which anolyte effluent containing hexavalent chromium, ammonium sulfate, and sulfuric acid, and catholyte effluent containing chromium sulfate, chromous sulfate and ammonium sulfate are produced, reducing the hexavalent chromium of the anolyte effluent to lower valence forms, and returning said reduced anolyte solution and said catholyte solution for admixture with the chrome liquor from which ferrous ammonium sulfate has been removed prior to the aging step.

REX R. LLOYD.  
JOE B. ROSENBAUM.  
VERNON E. HOMME.

References Cited in the file of this patent  
UNITED STATES PATENTS

| Number    | Name  | Date        |
|-----------|-------|-------------|
| 2,507,476 | Lloyd | May 9, 1950 |